

Aug. 26, 1941.

A. L. BOEGEHOOLD

2,253,502

MALLEABLE IRON

Filed Feb. 23, 1938



Inventor

Alfred L. Boegehold

By *Blackmores, Spencer & Black*  
Attorneys

## UNITED STATES PATENT OFFICE

2,253,502

## MALLEABLE IRON

Alfred L. Boegehold, Detroit, Mich., assignor to  
 General Motors Corporation, Detroit, Mich., a  
 corporation of Delaware

Application February 23, 1938, Serial No. 191,876

12 Claims. (Cl. 75—123)

This invention relates to a ferrous alloy and to a process of producing the same. More particularly the invention relates to irons suitable for making malleable iron castings and the manufacture thereof.

In my prior Patent 1,707,753, dated April 2, 1929, I have described and claimed certain improvements in the manufacture of white iron castings for malleabilizing whereby the time necessary to anneal the same may be materially reduced over the prior art practice. The patent teaches the use of a graphitizing agent, such as silicon, capable of promoting formation of temper carbon during annealing and an ingredient having the property of obstructing formation of flake graphite during solidification of the casting.

In my prior patent, the proportion of the graphitizing agent used was considerably larger than in the teachings of the prior art. This was made possible by the use of the ingredient having the property of obstructing formation of flake graphite during solidification of the casting.

I have now found a new method and new alloy for making white iron castings in which the time necessary to anneal the same may be materially reduced over the prior art practice. My invention comprises the addition of relatively small amounts of tellurium to irons containing larger amounts of graphitizing agents than ordinarily employed in the making of white irons suitable for malleabilizing. For example, silicon which is a graphitizing agent may not generally run much above 1.3% in the usual malleabilizing compositions without precipitating carbon in flake form upon solidification of the casting. Likewise, if other graphitizing agents are employed in amounts above that equivalent to about 1.3% silicon there is danger of precipitating graphite in flake form during solidification of the casting. In order to reduce the annealing time it is desirable that the graphitizing agent be present in such amount as to facilitate the formation of temper carbon during the annealing operation. My invention, therefore, comprises the use of small quantities of tellurium in iron compositions containing graphitizing agents in amounts equivalent in effect to 1.3%, or more, of silicon, which compositions are such that without the addition of tellurium grey iron would be formed upon solidification. In this way the amount of the graphitizing agent may be greatly increased and still attain white irons that may be readily annealed to form malleable iron.

I have found that tellurium has a powerful effect in preventing the formation of graphitic

carbon during solidification of the iron without retarding the action of the graphitizing agent in promoting formation of temper carbon during the subsequent annealing operation when the graphitizing agent is present in excess of an amount equivalent to about 1.3% silicon. This permits, if desired, the use of compositions of higher carbon contents, with the resulting advantages of greater fluidity of the iron, as well as the use of increased amounts of silicon which greatly reduces the time of annealing and also permits maintaining a higher silicon content in heavier sections than possible with ordinary iron without appearance of primary graphite.

15 The amount of tellurium necessary to stabilize the carbide in accordance with the invention is relatively small. Additions of tellurium to the molten metal as low as .0001% have an appreciable effect in light sections and, in general, amounts greater than .2% are unnecessary. Larger amounts than .2% may be used without detrimental effect on the malleabilized product; however, the higher amounts for most purposes are not recommended for the reason that the addition of tellurium to a molten ferrous metal bath results in fumes which are disagreeable and have a toxic effect. Consequently, the lower amounts of tellurium are less objectionable on this ground and for this reason are preferred. 20 For most purposes tellurium within the range .003% to .02% is entirely satisfactory for castings to be malleabilized having approximately 1.75% silicon.

25 The form in which the tellurium is added to the iron is immaterial to the invention. Metallic tellurium may be added to the molten iron coming from the cupola or electric furnace or, if desired, tellurium oxide may be added. The oxide is easily reducible and the iron reduces the same so that the tellurium alloys with the other constituents of the iron, as in the case of the addition of metallic tellurium. Other alloys or compounds containing tellurium may be used as the tellurium addition agent.

30 40 45 45 The following illustrative examples of practice in accordance with my invention may be given:

*Example 1*

An alloy containing 3.25% carbon, 2.25% silicon, .40% manganese and the balance iron with small amounts of impurities, such as phosphorus, sulphur, etc., normally present in cast irons was cast into a test bar  $\frac{1}{2}'' \times 1\frac{1}{2}'' \times 3\frac{1}{2}''$ . The structure of the iron in the bar was grey throughout. Metallic tellurium was added to a molten

iron of the same analysis to the amount of .10% of the alloy and cast into the same sized bar as before. The bar was white throughout. Annealing by heating the bar up to 1700° F. for about six hours substantially completely decomposed the iron carbide.

*Example 2*

An alloy containing 2.75% carbon, 1.75% silicon and the balance iron plus about .40% manganese, .07% phosphorus, and .11% sulphur, was cast into a test bar  $\frac{1}{2}'' \times \frac{1}{2}'' \times \frac{3}{2}''$ . The bar showed a grey structure throughout. The addition to the molten alloy of the following amounts of tellurium in the form of tellurium oxide resulted in white irons in the same size of test bars: .01%, .03%, .05%, .07%, .10%, .15%, .20%. Merely heating the bars to 1700° F. and cooling in the furnace resulted in a structure in which the iron carbide was substantially completely decomposed.

*Example 3*

An alloy was made containing 3.38% carbon, 1.91% silicon, and 0.40% manganese and the balance iron plus usual impurities such as phosphorus and sulphur in small amounts. To molten iron of the above analysis the following amounts of tellurium were added: .0001%, .0005%, .001%, .003%, .005%. The several irons were cast into wedge bars, tapering from a point to a 3" square section at the opposite end to determine the minimum amount of tellurium required. Fractures of these bars showed that the smallest quantity of tellurium had a measurable effect as a carbide stabilizing agent and indicated that .003% tellurium is sufficient for making white iron castings of compositions having a silicon content as high as 1.75% in castings having a cooling rate in the mold similar to a  $\frac{1}{8}''$  square by 7" long bar.

In general, as the proportion of silicon is increased or decreased the amount of tellurium that may be necessary to obtain white iron also will be increased or decreased, respectively. The same holds true for an increase or decrease in the carbon content of the iron. In the larger

amount present is thought to be somewhat less than the amounts added to the molten metal due to volatilization and with the larger amounts of tellurium addition the quantity present in the casting will be proportionately less than with the smaller additions. Qualitative tests show that in each case the solidified white iron casting contains tellurium. It has also been shown that upon remelting the iron, the fracture obtained upon recasting is typical of the one to which tellurium had been added which is proof that the tellurium remains in the iron in effective amounts.

The amounts of manganese and carbon in the iron may vary within ranges of known white irons suitable for annealing. If desired to increase the manganese content over the amount ordinarily used in standard compositions, i. e. about .40%, or to add other elements to the iron which would modify the physical properties of the annealed iron it may be necessary to raise or lower the amount of silicon present depending on whether the addition agent is a carbide stabilizer or a graphitizer. Elements in addition to silicon which may be classed as graphitizers include aluminum, barium, calcium, copper, lithium, magnesium, nickel, potassium, sodium, titanium and zirconium, while antimony, boron, chromium, manganese, molybdenum, sulphur, tin, tungsten and vanadium may be classed as carbide stabilizers. For example, if it is desired to obtain higher strength by increasing the manganese content over that of the standard composition, it may be necessary to slightly increase the silicon content to counteract the carbide stabilizing influence of the manganese. On the other hand if it is desired to add an element such as nickel or copper for increasing the tensile strength of the malleable iron it will be necessary to decrease the silicon content because these elements act as graphitizers in the same manner as silicon except that they are not as powerful. These examples, as well as others, are illustrated in the following table with an iron containing 2.75% carbon and show how the silicon should be adjusted to compensate for the addition of alloying elements.

|                                 | Percent C | Percent Si | Percent Te | Percent Mn | Percent S | Percent P | Percent alloy |
|---------------------------------|-----------|------------|------------|------------|-----------|-----------|---------------|
| Regular malleable.....          | 2.75      | 1.20       |            | .40        | .11       | .08       | -----         |
| Tellurium only.....             | 2.75      | 1.50       | .003       | .40        | .11       | .08       | -----         |
| Manganese increased.....        | 2.75      | 1.75       | .003       | 1.00       | .11       | .08       | -----         |
| Copper added.....               | 2.75      | 1.20       | .003       | .40        | .11       | .08       | 1.00 Cu       |
| Molybdenum added.....           | 2.75      | 1.75       | .003       | .40        | .11       | .08       | .50 Mo        |
| Copper and manganese added..... | 2.75      | 1.50       | .003       | 1.00       | .11       | .08       | 1.00 Cu       |

sections it may be desirable to increase the tellurium content somewhat.

As an example of the effect of tellurium and silicon on the fractures of test castings two inches in diameter and twelve inches long, attention is directed to the figure. The curves indicate the approximate amounts of the tellurium and silicon necessary to obtain white, mottled and grey irons. In addition to the tellurium and silicon the test specimens contained 2.75% carbon, .40% manganese, .12% sulphur, .07% phosphorus and the balance iron.

The amount of tellurium in the white iron casting prior to annealing is not known definitely. Quantitative tests for tellurium in the small amounts used herein are not accurate. Consequently, the exact amount of tellurium in the casting is not known. In each case the

One method for converting a grey iron melted in the cupola, into a white iron suitable for the manufacture of malleable iron, is to add steel. The amount of steel required depends upon the carbon and silicon content of the cupola grey iron. Even if it requires only 3 or 4% steel addition to convert a grey to a white iron, considerable labor is involved. About 1 to 2 ounces of tellurium per ton will serve substantially the same purpose at a considerably lower cost for labor.

The term "white iron casting" as used herein means a carbon containing iron free of appreciable amounts of carbon in flake form that characterizes ordinary grey iron castings. I do not intend the term to exclude annealable castings that may contain some nodular or temper carbon but contain substantially no flake carbon. White

iron as used commercially for the manufacture of malleable iron may have a small percentage of the structure containing flake graphite without detriment to the properties of the annealed product. These small areas are known as mottles and are similar to grey iron in structure.

All white iron castings are not suitable for the manufacture of malleable iron castings. A white iron casting containing no graphitizing element is unsuitable because the iron carbide will not decompose in a commercially useful period of time into iron and temper carbon upon subsequent annealing. Also, if the carbide stabilizer added to obtain a white iron of high silicon content is of such a nature that it makes the carbide so stable that it will not readily break down during annealing the iron is unsuitable for commercial malleabilizing. For example, chromium added to an iron with high silicon content may increase the tendency of the iron to solidify white but it also renders the carbides so stable they are very difficult to break down upon subsequent annealing. I have found that carbide stabilizers differ greatly in their relative stabilizing effect during solidification of the iron compared to their stabilizing effect during the annealing operation. Whereas chromium increases somewhat the power of an iron to solidify white, tellurium is exceedingly powerful in this property. On the other hand chromium is powerful in preventing decomposition of iron carbide at annealing temperature even when the silicon content is high while tellurium has very little carbide stabilizing effect at the annealing temperature when 1.50% or more silicon is contained in the iron. In this respect tellurium is especially advantageous. In the drawing it is shown that an iron with 2.75% carbon and 1.75% silicon solidifies grey in a two inch round casting and is useless for making malleable iron, whereas the addition of .01% tellurium to this iron by its effect on the carbide makes the iron solidify white and yet it will anneal so rapidly because of the 1.75% silicon that the first stage of annealing is complete in three hours as compared to ten hours for malleable iron of the usual composition containing about 1.20% silicon.

Annealed castings in accordance with my invention show the same microstructure that characterizes malleable castings made by prior art practices and appear in all respects to be adapted for use wherever malleable castings may be employed.

My invention is not limited to irons having carbon contents suitable for ordinary malleable castings. For example, it may be desired to cast ingots eight or ten inches in diameter containing as low as 1.5% carbon, which, after partial graphitization or annealing may be rolled into bars, or pierced and drawn into tubes. Small additions of tellurium permits the use of higher silicon content without the appearance of flake graphite in the ingot as cast. This facilitates the annealing or graphitization and may be useful in modifying the physical properties of the final product due to the alloying effect of the silicon.

It will be understood that various modifications and changes may be made in the embodiment of my invention set forth herein by skilled metallurgists without departing from the principle and spirit of my invention and I do not desire to limit the patent granted thereon except as necessitated by the prior art.

I claim:

1. An annealable white iron casting substantially free from flake graphite and characterized by the rapidity with which it can be annealed to form malleable iron containing, at least 1.50% carbon, at least about .40% manganese, a graphitizing agent equivalent in effect to approximately 1.3% or more of silicon and a small but effective amount of tellurium up to about .2% sufficient to obstruct formation of flake graphite during solidification of the casting without appreciably retarding the decomposition of iron carbide during annealing.
- 15 2. An annealable casting as in claim 1 in which the carbon content is within the approximate range 2-3.50% and the graphitizing agent is present in amount equivalent in effect to approximately 1.3-2.25% of silicon.
- 20 3. A white iron casting characterized by the rapidity with which it can be annealed to form malleable iron, composed of the following elements as essential constituents in substantially the proportions stated:

|           | Per cent  |
|-----------|-----------|
| Carbon    | 1.50-3.50 |
| Silicon   | 1.30-2.25 |
| Manganese | .40-1.00  |

a small but effective amount of tellurium up to about .2% sufficient to obstruct formation of flake graphite during solidification of the casting without appreciably retarding the decomposition of iron carbide during annealing, balance substantially all iron.

- 35 4. A white iron casting substantially free of flake graphite characterized by the rapidity with which it can be annealed to form malleable iron containing approximately 1.50-3.50% carbon, approximately 1.30-2.25% silicon, approximately .40-1.00% manganese and a small but effective amount of tellurium up to about .2% sufficient to obstruct formation of flake graphite during solidification of the casting without appreciably retarding the decomposition of iron carbide during annealing to form malleable iron.

- 50 5. A white iron casting substantially free of flake graphite characterized by the rapidity with which it can be annealed to form malleable iron containing approximately 1.50-3.50% carbon, a graphitizer equivalent in effect to approximately 1.30-2.25% silicon, approximately .40-1.00% manganese and a small but effective amount of tellurium up to about .2% sufficient to obstruct formation of flake graphite during solidification of the casting without appreciably retarding the decomposition of iron carbide during the annealing to form malleable iron.

- 60 6. An annealable white iron casting substantially free from flake graphite characterized by the rapidity with which it can be annealed to form malleable iron containing, at least 1.50% carbon, a graphitizing agent equivalent in effect to at least 1.3% silicon and a small but effective amount of tellurium up to about .2% sufficient to obstruct formation of flake graphite during solidification of the casting without appreciably retarding the decomposition of iron carbide during the annealing to form malleable iron.

- 65 7. An annealable white iron casting substantially free from flake graphite and characterized by the rapidity with which it can be annealed to form malleable iron composed as follows: approximately 2.00-3.50% carbon, approximately

1.30-2.25% silicon, approximately .40-1.00% manganese, a small but effective amount of tellurium up to about .2% sufficient to obstruct formation of flake graphite during solidification of the casting without appreciably retarding the decomposition of iron carbide during annealing, and the balance substantially all iron.

8. An annealable white iron casting substantially free from flake graphite and characterized by the rapidity with which it can be annealed to produce malleable iron containing at least 1.50% carbon, at least 1.3% silicon, and a small but effective amount of tellurium up to about .2% sufficient to obstruct formation of flake graphite during solidification of the casting without appreciably retarding the decomposition of iron carbide during annealing to form malleable iron.

9. An annealable white iron casting substantially free from flake graphite containing, at least 1.50% carbon, at least about .40% manganese, a graphitizing agent equivalent in effect to approximately 1.3% or more of silicon and a small but effective amount of tellurium up to about .2% sufficient to obstruct formation of flake graphite during solidification of the casting.

10. As an article of manufacture, a malleable-ized cast iron having temper carbon and containing 1.50% to 3.50% carbon, a graphitizing agent

equivalent in effect to 1.30% to 2.25% silicon, and tellurium in small but effective amount not to exceed .2%.

11. Process of making a malleable cast iron product comprising casting a fused mixture containing carbon in excess of 1.5%, a graphitizing agent equivalent in effect to at least 1.3% silicon and iron substantially the remainder, in the presence of a small but effective amount of tellurium sufficient to substantially obstruct separation of carbon in flake form during solidification, said amount being between .0001% and .2% of the mixture, thereby producing a white cast iron body, and then subjecting said body to an annealing treatment to cause separation of at least a portion of the carbon as temper carbon.

12. Process of making a malleable cast iron article comprising casting a mixture containing 1.50%-3.50% carbon, 1.30%-2.25% silicon and not less than about 94% iron, in the presence of a small but effective amount of tellurium, from .0001% to .2% of the mixture, sufficient to obstruct formation of carbon in flake form during solidification, thereby producing a white cast iron article, and then annealing the article under conditions to cause separation of at least a portion of the carbon as temper carbon.

ALFRED L. BOEGEHOOLD.